

## UNITED STATES PATENT OFFICE

2,029,382

## PROCESS FOR PRODUCING HIGH MOLECULAR WEIGHT COMPOUNDS FROM PETROLEUM OIL

David R. Merrill, Long Beach, Calif., assignor to  
Union Oil Company of California, Los Angeles,  
Calif., a corporation of California

No Drawing. Application November 20, 1933,  
Serial No. 698,878

8 Claims. (Cl. 196—13)

The present invention relates to a process for producing lubricating oils of low pour point and green fluorescence. In particular, the invention relates to a process for producing pour point depressing agents adapted to be added to lubricating and other oils in order to lower the pour point of such oils.

It has been found that heavy asphaltic bodies from cracked residuum contain valuable materials which, when added to lubricating oils, impart a green bloom or fluorescence and depress the pour point of oils containing wax. As is well known, lubricating oils are desirable which possess a low pour point, i. e. do not congeal at the lower temperatures. Oils which contain paraffin or wax solidify at the lower temperatures and will not flow. To overcome this undesirable characteristic of waxy oil, it has been customary in the art of producing lubricating oils to remove the wax or paraffin from the oil to as great an extent as is feasible. This is usually accomplished by chilling the oil preferably in the presence of a solvent in order to precipitate the wax and then separating the precipitated wax from the oil solvent solution by settling, centrifuging or filtering. The solvent is then removed from the dewaxed lubricating oil by distillation.

Another desirable characteristic of lubricating oil is a low temperature viscosity susceptibility, i. e. a minimum change in viscosity with a given change in temperature. Lubricating oils produced from paraffin base crudes exhibit a low temperature viscosity susceptibility, whereas those produced from asphaltic base crudes as distillates exhibit a relatively high temperature viscosity susceptibility. I have observed that the removal of wax from oils containing the same increases the temperature viscosity susceptibility of the oil; in other words, waxes per se have especially low temperature viscosity susceptibility and impart to oils containing them a low temperature viscosity susceptibility. Consequently, their removal from oil is to be considered harmful from the standpoint of impairment of the temperature viscosity susceptibility of the oil.

In order to permit oils having high pour points to flow at the lower temperatures without effecting complete removal of the wax or paraffin or other substances in the oil which cause it to congeal under ordinary conditions of high temperatures, it has been proposed to add to the lubricating oil, petroleum fractions containing high molecular weight bodies which are very effective in depressing the pour point or congealing point of the oil and which also impart to lubricating oils

produced from distillates or for other reasons deficient in green bloom, a rich green fluorescence characteristic of lubricating oils produced from paraffin base crude oils.

One of the recent methods proposed for producing these petroleum fractions is to obtain a cracked residue such as the cracked residuum produced by cracking gas oil to produce gasoline in a Cross cracking process at a maximum pressure of 800 lbs. and a maximum temperature of 10 880° F. The residue obtained as the bottoms from the flashing drum in which gasoline and cycle stock are removed by distillation is then treated for the recovery of the high molecular weight and complex compounds comprising the 15 pour point depressants. The recovery of these complex compounds from cracked residuum consists in first distilling the residue to remove the lighter constituents and to leave a high melting point cracked residuum pitch as a distillation bottom and then extracting the cracked residuum pitch with a suitable solvent in which the carbonaceous and coke-like bodies present in the cracked residuum pitch are not soluble but in which the desired pour point depressing agents 20 and wax crystallization inhibitors are soluble. A solvent solution of pour point depressing agents 25 is separated from the coke-like bodies by such methods as settling, centrifuging or filtering. One of these solvents comprises a lubricating oil or a 30 lubricating oil stock, that is, an oil possessing physical characteristics similar to the oil to be treated for pour point depressing. A concentrated oil solution of the active pour point depressing agents is made which may be added to 35 the oil to be treated for pour point depressing. The concentrated solution is then treated with concentrated sulphuric acid of, say, 98% strength, neutralized with caustic alkali and clay treated with decolorizing clay by methods conventional 40 in the art, or may be treated with clay alone, without a prior acid treatment.

The present invention relates in part to an improvement on the foregoing process for producing pour point depression agents adapted to 45 be added to oils containing wax. I have discovered that when the concentrated solution of oil containing the pour point depressing agents is treated with concentrated sulphuric acid as aforesaid, a large proportion of the valuable components which impart a green bloom to lubricating oils and lower the pour point of waxy oils are lost to the acid sludge. The concentrated sulphuric acid appears not only to attack the undesirable and unstable components but also 50 55

attacks the valuable high molecular weight compounds and yet it is entirely necessary to effect a treatment of the crude material in order to produce a product of satisfactory refinement as regards color and stability.

It is, therefore, an object of my invention to improve upon the aforesaid process for producing pour point depressing and green bloom compounds adapted to lower the pour point and impart a green fluorescence to lubricating oils and the like.

Another object of my invention resides in providing a process wherein increased yields of pour point depressing agents may be recovered from cracked residuum pitches and the like containing such agents.

It is a particular object of my invention to restrict the activity of the acid employed to treat the pour point depressing agent and thus prevent a large proportion of the valuable pour point depressing agents present in the crude material from being attacked by the acid and thus lost to the acid sludge and yet to produce pour point depressing agents of satisfactory refinement.

25 Briefly stated, my invention relates to a process for producing high molecular weight compounds from cracked residuum which are capable of lowering the pour point of oils and imparting a green fluorescence to lubricating oils which comprises first extracting a crude pour point depressant from a cracked residuum pitch and then treating it in the presence of a solvent with acid, such as sulphuric acid. The invention includes the extraction of a crude pour point depressant and 30 green bloom compounds from cracked residuum pitches and the like by means of a solvent capable of dissolving the pour point depressant and green bloom compounds but capable of dissolving only limited asphaltic, carbonaceous and 35 coke-like materials, and subsequently treating the pour point depressant and green bloom compounds with sulphuric acid while the compounds are dissolved in a solvent.

One of the particular features of my invention 40 comprises the treatment of the extracted pour point depressing agents with acid in the presence of a highly aromatic solvent.

More particularly stated, my invention comprises a process for producing pour point depressants in which a cracked petroleum residuum is first reduced to a pitch-like consistency and then the pitch is mixed with a solvent capable of dissolving the pour point depressing agents present in the cracked residuum pitch but to leave for 45 the most part as undissolved fractions the asphaltic and coke-like materials resulting from the cracking operation, then separating the latter from the solvent solution and acid treating the dissolved fractions in the presence of a highly aromatic solvent such as benzene.

I have discovered that when the crude pour point depressing agent, such as the extract of a cracked residuum pitch, is acid treated in the presence of a highly aromatic solvent which has 50 a high solvent power for the high molecular weight compounds present in cracked residuum pitches and which comprise the pour point depressing agents, the action of the acid is restricted to the more reactive undesirable constituents 55 present in the crude pour point depressing agent leaving unattacked the valuable pour point depressing agents. When the crude material is treated directly with sulphuric acid or in the presence of a solvent other than the highly aromatic solvent, a considerable amount of the val-

able constituents are lost to the acid sludge. The use of a highly aromatic solvent appears to take the high molecular weight compounds into a true solution rather than a colloidal solution and thus the action of the sulphuric acid is restricted to the more reactive bodies present in the solution but not the more colloidal hydrocarbons present in the cracked residuum extract.

60 The high molecular weight compounds comprising the valuable pour point depressing agents are preferably produced from asphaltic residues, particularly cracked residues, such as those resulting from the cracking of kerosene, gas oil or other cracking stocks in the production of cracked gasoline, although they may be produced by cracking petroleum residues or heavy oils to reduce their viscosity. In general, the poor point depressants are preferably produced from stocks having a sufficient quantity of high molecular weight bodies and resinous materials.

65 The lower molecular weight hydrocarbons present in the cracked residuum are of little value in depressing the pour point of wax-containing oil. Therefore, the extracts which are produced from moderately viscous cracked residua are, in general, less effective in depressing the pour point of oils than are the extracts which are produced from the cracked residuum pitches. Also, the lighter fractions of the cracked residua are generally less stable in character than the lubricating oil to which it is desired to add the pour point depressing agents. Moreover, the lighter constituents of the residua often have high solvent properties for the asphaltic and coke-like material and may interfere with the precipitation of such impurities during extraction with oils as will be described. Therefore, I prefer to remove the light constituents present in the cracked residuum prior to the extraction step with the solvent.

70 The removal of the lower molecular weight hydrocarbons may be effected by steam distillation, preferably under vacuum, until a pitch remains as a distillation bottom which has a high melting point, i. e. in excess of 200° F. Lubricating oil or lubricating oil stock is then added to the pitch while still hot in the still and the mass is thoroughly agitated with steam. After thorough agitation, the mass is allowed to remain in a quiescent state in the still until the black carbonaceous and coke-like bodies have settled out.

75 The type of oil used for the extraction step will be governed by the use to which the concentrated oil solution of active pour point depressant ingredients is to be employed. Generally, it will be preferable to use an oil for the extraction step which has physical characteristics similar to the oil to be treated for pour point depression, although other solvents may be employed which have a preferential solubility for the high molecular weight hydrocarbons present in the cracked residuum pitch to leave as undissolved fractions the carbonaceous and coke-like materials. As solvents capable of dissolving the high molecular weight pour point depressants from the asphaltic 80 carbonaceous and coke-like materials, I may employ in addition to the lubricating oil or lubricating oil stock mentioned, naphtha, gasoline, kerosene, gas oil, fuel oil, alcohols, such as butyl alcohol, ketones, such as acetone, and esters, such as methyl formate. The amount of oil or solvent used in the extraction step may vary, depending upon the type of solvent employed and the character of the material containing the pour point depressants. However, I find that about 4 to 7

volumes of lubricating oil to one volume of the pitch gives very satisfactory results.

After settlement of the coke-like materials, the concentrated lubricating oil solution of active pour point depressant ingredients is decanted away and is ready for acid treatment. This solution is then dissolved in a highly aromatic solvent and treated with sulphuric acid of 93% or less strength. As solvent, I may employ benzene, toluene, xylene, heavy solvent naphtha from coal tar, highly aromatic solvents produced from the liquid sulphur dioxide treatment of light oils, such as Edeleanu extract, chlorinated solvents such as carbon tetrachloride, ethylene dichloride or trichloride, carbon disulphide and the like. The amount of solvent used for admixture with the pour point depressant is more or less elastic and will depend upon the type of aromatic solvent added and the character of the pour point depressant. In general, a sufficient amount is employed to reduce the viscosity of the mass in order to permit acid sludge produced by the acid treatment to settle from solution. I may employ from one to three volumes of the solvent to one volume of the concentrated oil solution of pour point depressing ingredients. When solvents other than the lubricating oil or lubricating oil stock are employed for extracting the high molecular weight hydrocarbons or materials from the cracked residuum pitch and such solvents may interfere with the acid treatment in the presence of a highly aromatic solvent such solvents may be removed, as, for example, by distillation prior to the addition of the highly aromatic solvent to the pour point depressing agent. However, in the case of the lubricating oil, I prefer to add the aromatic solvent to the concentrated solution of pour point depressant and then acid treat the mixture. The acid treated mixture may then be distilled to remove the aromatic solvent leaving as a distillation bottom a concentrated oil solution of acid treated pour point depressing ingredients which may be added to the oil to be treated for pour point depression.

The amount and concentration of acid should be carefully restricted in order to prevent removal as acid sludge, valuable components of pour point depressant character. The amount and concentration of acid will depend upon the character of the high molecular weight hydrocarbons of pour point depressants to be treated. In general, I may employ acid of 93% or less strength in an amount of, for example, 30 lbs. per barrel based on the concentrated oil solution of the high molecular weight hydrocarbons, although I may use very small proportions of the more concentrated acids. After the acid treatment, the solvent solution may be neutralized with aqueous alkali or by dry methods, such as treatment with fuller's earth or other clays and I may further purify by clay treatment as by percolation of the solvent solution before recovering the product by evaporation of the solvent.

In producing my pour point depressing agent from recycled cracked gas oil residuum, I prefer to proceed as follows, although this is not to be considered as limiting my invention:

A cracked residuum, such as one obtained from cracking in recycling operations, a gas oil fraction distilled from a San Joaquin Valley crude to produce cracked gasoline, is reduced by fire and steam until a hard pitch is produced having a melting point of approximately 300 to 400° F. The molten pitch in the still is then thoroughly

mixed by steam agitation at a temperature of approximately 450 to 500° F. with lubricating oil in the proportion of one volume of pitch to five volumes of lubricating oil. The mixture is then allowed to settle for a period of ten to twelve hours with slow cooling after which the supernatant layer of oily solution is decanted away from the black carbonaceous bodies. This concentrated solution of pour point depressing ingredients is then mixed with an aromatic solvent such as benzene in the proportion of one volume of the concentrated oil solution to two volumes of benzene. The mixture is then acid treated with about 25 lbs. of 93% sulphuric acid per barrel of the concentrated oil solution. The acid sludge is removed and the mixture is then neutralized with caustic soda and the benzene is removed by distillation, leaving as a distillation bottom a purified oil concentrate of pour point depressants. If a relatively light color is desired, the concentrate is then clay treated with about 5% of decolorizing clay. These materials may then be added to the oil having a high congealing temperature or pour point in an amount sufficient to lower the congealing temperature or pour point to the desired value.

The amount of this concentrated solution of pour point depressing agents or compounds which must be added to the waxy oil to lower its pour point to the desired value will vary; however, in most instances the addition of about 2% by volume of the concentrate to the oil will be sufficient. For example, by adding 2% of the agent to a waxy lubricating oil having a pour point of approximately 40° F., the pour point may be lowered to 0° F. When the oil has a high congealing temperature due to large amounts of wax, it may be necessary to increase this amount to 3 to 5%.

While the cracked residua referred to in the above examples have been obtained by cracking distilled products, such as gas oil or cycle stock, the cracked residua obtained from the conversion of crude oils or fuel oils by the various cracking processes now known also contain large amounts of pour point reducing agents. The cracked residua which I employ as a source of pour point depressing agents are not limited to any particular type of cracking stock or to any method of operation of the cracking process because substantially all cracked residua, regardless of the source or method for their production, have been found to contain pour point reducing agents which appear to have been formed simultaneously with the gasoline or gas in the conversion process. The exact concentration of the pour point depressing agents, however, is dependent on the cracking conditions and in the charging stock with the more severe cracking conditions and highly aromatic or naphthenic charging stocks generally favoring a higher yield of pour point depressing agents.

If desired, the pour point depressing agent may be produced by distilling the cracking residuum with fire and steam until a pitch is left in the still having a melting point above 300° F. and then collect the heavy distillate produced upon further distillation of the pitch in the still. The distillate so produced possesses pour point depressing characteristics, and when acid treated in the presence of an aromatic solvent and the solvent removed, it may be employed to lower the congealing point of oil. However, such distillates obtained from cracked pitches are not as effec-

tive as the material extracted from the pitches by means of suitable solvents.

While cracked residua have been found to be highly satisfactory sources of these pour point depressing agents, I have found that these materials may also be produced from crude oil residues; for example, asphalt base crude oil which is relatively free from wax may be distilled until a residue is obtained having a melting point between 200 and 350° F. which is then extracted in the same manner as previously described for the production of agents which are affected in lowering the pour point of oil. These materials are then acid treated in the presence of an aromatic solvent as above described.

When these heavy hydrocarbons recovered from residuum or cracked pitch by the methods hereinabove described are blended with oil and especially lubricating oil, the resultant pour point is depressed and the blended oil is characterized by a rich green fluorescence which is characteristic of lubricating oil produced from paraffin base crude oil.

My invention is also useful in conjunction with the production of low pour point, high grade fuel oils of light color of either the distillate or residual type. Fuel oils which congeal at moderate temperatures and which cannot be transported through pipe lines or withdrawn from storage during cold weather without heating to maintain a temperature well above the congealing point of the oil can be made to flow at much lower temperatures by the addition of the herein described pour point depressing agent. When it is desired to lower the pour points of such oils as gas oil or Diesel fuel oil, I find it desirable to employ a light solvent oil having characteristics similar to the gas oil and Diesel fuel oil itself to extract the high molecular weight depressing agents from the stock containing the same. In such cases, it is unnecessary to reduce the cracked residue to a pitch before the extraction. The extract so obtained is then acid treated in the presence of a highly aromatic solvent, neutralized and possibly clay treated, and then added to the gas oil or Diesel fuel oil in an amount sufficient to produce the desired depression of the pour point.

By "pour point" is meant the temperature of 5° above the test temperature at which an oil ceases to flow as determined by the American Society of Testing Materials, Method D-97-30. The melting points stated herein are determined by the Ball and Ring Method of the same society, Method D-36-26.

By the terms "paraffin" or "wax", I mean to designate those substances which cause hydrocarbon oil to cease to flow upon the lowering of the temperature.

It is to be understood that the above description of my invention is merely illustrative of preferred embodiments of my invention of which many variations within the scope of the following claims may be made by those skilled in the art without departing from the spirit thereof.

63 I claim:

1. A process for the production of high molecular weight hydrocarbons which comprises commingling a cracked residuum pitch with a solvent capable of dissolving high molecular weight hydrocarbons from said pitch but to leave an insoluble residue, separating a solvent solution of high molecular weight hydrocarbons from the insoluble residue, commingling said high molecular weight hydrocarbons with an aromatic solvent, treating said high molecular weight hydrocarbons with an aromatic solvent with acid and separating said aromatic solvent from said acid treated high molecular weight hydrocarbons.

and aromatic solvent with acid and separating said aromatic solvent from said acid treated high molecular weight hydrocarbons.

2. A process for the production of high molecular weight hydrocarbons which comprises distilling a cracked residuum to produce a pitch of high melting point, commingling said pitch with an oil to dissolve high molecular weight hydrocarbons from said pitch but to leave an insoluble residue, separating the oil solution of high molecular weight hydrocarbons from the insoluble residue, commingling said oil solution with a highly aromatic solvent, treating said solution with sulphuric acid of such concentration and in an amount to remove undesirable reactive bodies and separating said highly aromatic solvent from said acid treated high molecular weight hydrocarbons.

3. A process for the production of high molecular weight hydrocarbons which comprises distilling a cracked residuum to produce a pitch of high melting point, commingling said pitch with an oil at an elevated temperature to dissolve high molecular weight hydrocarbons from said pitch but to leave an insoluble residue, separating the oil solution of high molecular weight hydrocarbons from the insoluble residue, commingling said oil solution with a highly aromatic solvent, treating said solution with sulphuric acid of such concentration and in an amount to remove undesirable reactive bodies and separating said highly aromatic solvent from said acid treated high molecular weight hydrocarbons.

4. A process for the production of high molecular weight hydrocarbons which comprises distilling a cracked residue to a pitch-like consistency of high melting point, commingling said pitch at a temperature of approximately 400 to 450° F. with an oil capable of dissolving high molecular weight hydrocarbons present in said pitch but to leave an insoluble residue, separating the oil solution of high molecular weight hydrocarbons from the insoluble residue, commingling said oil and high molecular weight hydrocarbons with an aromatic solvent, treating said mixture of high molecular weight hydrocarbons dissolved in said oil and aromatic solvent with sulphuric acid and subsequently separating said aromatic solvent from said acid treated oil and high molecular weight hydrocarbons.

5. A process for the production of high molecular weight hydrocarbons which comprises distilling a cracked residue to a pitch-like consistency of high melting point, commingling said pitch at a temperature of approximately 400 to 450° F. with an oil capable of dissolving high molecular weight hydrocarbons present in said pitch but to leave an insoluble residue, separating the oil solution of high molecular weight hydrocarbons with benzene, treating said mixture of high molecular weight hydrocarbons dissolved in said oil and benzene with sulphuric acid and subsequently separating said benzene from said acid treated oil and high molecular weight hydrocarbons.

6. A process for the production of high molecular weight hydrocarbons which are adapted to lower the pour point of oils or to impart green fluorescence to oils which comprises commingling a cracked pitch with a substantially non-aromatic solvent to dissolve high molecular weight hydrocarbons contained in said pitch but to leave an insoluble residue, separating the solution of non-aromatic solvent and high molecular weight hydrocarbons from the insoluble residue and com-

mingling said mixture with a solvent having a high solvent power for desirable high molecular weight hydrocarbons so that subsequent action with acid is restricted to unstable reactive bodies contained in the high molecular weight hydrocarbons, treating said mixture with acid to remove the undesirable unstable reactive bodies and subsequently separating the solvent from the acid treated desirable high molecular weight hydrocarbons.

10 7. A process for the production of high molecular weight hydrocarbons which comprises commingling a cracked pitch with a lubricating oil to dissolve crude high molecular weight hydrocarbons contained in said pitch but to leave an insoluble residue, separating the solvent solution

of high molecular weight hydrocarbons and oil from the insoluble residue, commingling said solution with a solvent selected from the class consisting of benzene, toluene, xylene, heavy solvent naphtha obtained from coal tar, liquid sulphur dioxide soluble hydrocarbons, carbon tetrachloride, ethylene dichloride, ethylene trichloride and carbon disulphide, treating the solution of high molecular weight hydrocarbons, oil and solvent with sulphuric acid to remove the undesirable unstable reactive bodies and separating the solvent from the acid treated high molecular weight hydrocarbons and oil.

15 8. A process as in claim 7 in which the strength of sulphuric acid employed does not exceed 93%. DAVID R. MERRILL.